

Jan. 7, 1936.

O. S. BUCKNER

2,027,087

ABRASIVE SHEET AND PROCESS OF MAKING THE SAME

Filed Oct. 3, 1928



Inventor.  
Orville S. Buckner  
by L. M. Hammann  
Atty.

## UNITED STATES PATENT OFFICE

2,027,087

ABRASIVE SHEET AND PROCESS OF  
MAKING THE SAMEOrello S. Buckner, Westboro, Mass., assignor to  
Behr-Manning Corporation, Troy, N. Y., a cor-  
poration of Massachusetts

Application October 3, 1928, Serial No. 310,058

8 Claims. (Cl. 91—68)

This invention relates to a modified form of the invention disclosed in my issued Patent 1,930,788, dated October 17, 1933, which relates to abrasive or attrition tools and methods of making the same, and in the construction of which the elongated grains of abrasive material are electrically positioned, so that they are bonded in approximately perpendicular relation to the working face of the tool.

10 The present invention relates, more specifically to an application of the generic invention to the production of abrasive or attrition sheets and has for its object the production of a sheet of this character which has the essential characteristics of the abrasive tools previously disclosed in said application and to a method of making the same which will be commercially successful.

I accomplish these objects in the manner hereinafter described and illustrated in the accompanying drawing in which:

Fig. 1 is a side elevation of the essential features of an apparatus which I preferably employ in performing the process of making attrition sheets.

25 Fig. 2 is a plan view thereof.  
Fig. 3 is a sectional view of the finished product.

In carrying out the method of the present invention, in order to make the abrasive material responsive to a magnetic field the abrasive grains 30 are coated with a moist adhesive, then are mixed with finely pulverized iron or steel, and then the adhesive is permitted to dry, so that the grains become coated with a magnetic substance. As some of the grains are likely to adhere to each 35 other, this adhesion must then be broken, and this may be accomplished in various ways, as by working the same through a wire screen of suitable mesh.

As thus prepared, the grains are applied to 40 sheets of suitable material in the following manner; the apparatus which is preferably employed comprising an electromagnet 1 of straight cylindrical form having the faces of its ends, which form the poles, disposed in planes perpendicular to the central axis of the magnet, the latter being disposed perpendicularly so that said faces will be horizontal. A table 2 of thin brass, or similar non-magnetic substance is disposed on the top end of the magnet and is provided with 45 a series of suitably arranged guide rolls 3 at its edges beneath which the sheets to be coated are passed. A receptacle 4 having a wire mesh bottom 5 is mounted horizontally directly over the magnet, suitable agitating means 6 being provided for moving the receptacle horizontally,

The paper, cloth, or other form of sheet material 7 is coated with a suitable adherent as glue and is then fed over the table 2 beneath rolls 3, to hold it flat, while resting on its surface. The abrasive grains which have previously been coated with the finely divided magnetic dust are placed in the receptacle 4, which is then agitated in any suitable manner as by the reciprocating means indicated, so that the grains will be showered onto the adhesively coated sheet as it 10 is fed over the pole of the magnet. The lines of force of the magnet passing from one pole to the other have principally an approximately vertical direction close to the surface of the sheet and will cause the magnetically coated grains, 15 most of which will be somewhat elongated, or will have one dimension substantially greater than the dimension at right angles thereto, to be polarized as they fall, so that, assuming the pole at the top of the magnet is positive, the negatively magnetized ends of the grains will be attracted and the positive ends repulsed, and they will be turned while falling into approximately perpendicular relation to the face of the sheet, with the result that the ends of the elongated 20 grains will penetrate the adhesive coating and will stand upright therein, as indicated in Figs. 1 and 3. As hereinafter explained, it is an object of the invention to provide a final product in which the grains are substantially all arranged 25 with their major axes substantially perpendicular to the carrier sheet and the further operations are performed to provide a material having these characteristics.

The adhesive will then be permitted to set while 30 still held horizontally and, after this has occurred, the surplus grains which did not penetrate or touch the adhesive will be shaken off.

The material after these operations have been performed does not have the arrangement of the 35 particles effected by the magnetic field appreciably disturbed. In other words, the resulting abrasive sheet will have practically all the elongated abrasive grains thereon oriented to stand perpendicularly, so that the abrading efficiency 40 of the sheet will be much greater than if they lie flatwise of the sheet, on account of the superior cutting qualities of the ends of the abrasive grains, as compared with the sides thereof. The coating of abrasive grains, which is applied to 45 the sheet will also be of greater thickness than it would be if the grains were not positioned on the sheet in perpendicular relation thereto.

I claim:

1. The method of making attrition sheets 50

which consists in placing a sheet having an adhesive surface in a magnetic field, so that the lines of force pass approximately perpendicularly therethrough and showering magnetically coated 5 elongated grains of abrasive material onto said surface.

2. The method of making attrition sheets which consists in providing a sheet of suitable material with an adhesive surface, showering 10 granular abrasive material containing a substantial portion of elongated grains onto said surface and simultaneously magnetically positioning said elongated grains, as they fall, in approximately perpendicular relation to said surface, so that the 15 end portions of said grains may penetrate said surface and become bonded therein in approximately perpendicular relation thereto.

3. The method of making attrition sheets which consists in covering one surface of a sheet 20 with a suitable adhesive material, passing the sheet while held horizontally with its adhesive side uppermost through the field of a magnet so that the lines of force thereof pass mainly approximately perpendicularly through the sheet 25 and showering magnetically coated elongated abrasive grains through the field of the magnet onto said surface.

4. The process of making abrasive material which comprises providing a magnetic field, feeding 30 a carrier having a surface coated with adhesive through said field with the lines of force of the field at an angle to the adhesively coated surface of the carrier, causing abrasive particles of a character responsive to magnetic action 35 to be deposited on the carrier, utilizing the field to arrange the particles on the adhesive surface with their major axes substantially perpendicular to the adhesive surface, and conducting the abrasively coated carrier away from the field as the 40 particles are deposited thereon.

5. The process of making abrasive material which comprises providing an electromagnetic field, feeding a carrier having a surface coated with adhesive through said field with the lines of 45 force of the field at an angle to the adhesively coated surface of the carrier, causing abrasive particles of a character responsive to electromagnetic action to be deposited on the carrier, utilizing the field to arrange the particles on the adhesive surface with their major axes substantially perpendicular to the adhesive surface, and conducting the abrasively coated carrier away 50

from the field as the particles are deposited thereon.

6. The process of making abrasive material which comprises providing a magnetic field, feeding a carrier having a surface coated with adhesive through said field with the lines of force of the field at an angle to the adhesively coated surface of the carrier, causing abrasive particles of a character responsive to magnetic action to be deposited on the carrier, utilizing the field to 10 arrange the particles on the adhesive surface with their major axes substantially perpendicular to the adhesive surface, conducting the abrasively coated carrier away from the field as the particles are deposited thereon, and performing the 15 finishing operation to produce a material having the particles with their major axes substantially perpendicular to the adhesive surface.

7. The process of making abrasive material which comprises providing an electromagnetic field, feeding a carrier having a surface coated with adhesive through said field with the lines of force of the field at an angle to the adhesively coated surface of the carrier, causing abrasive particles of a character responsive to electromagnetic action to be deposited on the carrier, utilizing the field to 20 arrange the particles on the adhesive surface with their major axes substantially perpendicular to the adhesive surface, conducting the abrasively coated carrier away from the field as the particles are deposited thereon, and performing the 25 finishing operation to produce a material having the particles with their major axes substantially perpendicular to the adhesive surface.

8. The process of making abrasive material which comprises providing a magnetic field, feeding a carrier having a surface coated with adhesive through said field with the lines of force of the field at an angle to the adhesively coated 30 surface of the carrier, causing abrasive particles of a character responsive to magnetic action to be deposited on the carrier, utilizing the field to arrange the particles on the adhesive surface with their major axes substantially perpendicular to the adhesive surface, conducting the abrasively coated carrier away from the field as the particles are deposited thereon, and permitting the adhesive to set while maintaining the carrier substantially horizontal.

ORELLO S. BUCKNER.

35

40

45

50